

W. M. GROSVENOR,  
PROCESS OF GLUING WOOD,  
APPLICATION FILED JAN. 16, 1918.

1,299,705.

Patented Apr. 8, 1919.

*Fig. 1.*



*Fig. 2.*



Inventor

William M. Grosvenor,  
By his Attorney  
Gorham Crosby.

# UNITED STATES PATENT OFFICE.

WILLIAM M. GROSVENOR, OF NEW YORK, N. Y., ASSIGNOR TO PERKINS GLUE COMPANY,  
A CORPORATION OF PENNSYLVANIA.

## PROCESS OF GLUING WOOD.

1,299,705.

Specification of Letters Patent.

Patented Apr. 8, 1919.

Application filed January 16, 1918. Serial No. 212,045.

*To all whom it may concern:*

Be it known that I, WILLIAM M. GROSVENOR, a citizen of the United States, and a resident of New York city, in the county of New York and State of New York, have invented certain new and useful Improvements in Processes of Gluing Wood, of which the following is a specification.

My invention relates to improvements in processes for gluing wood and is particularly applicable to the gluing up of wood panels, veneers and joints for furniture and similar work. For many years animal glue was the only glue generally used for this purpose, but this has now been largely supplanted by vegetable glue, made from a starchy carbohydrate base, water and a solvent. In the making of such vegetable glue, cassava starch has been generally used, and it has generally been found necessary to hydrolyze or degenerate the starch a certain extent before dissolving it in the water with the solvent, and in spite of such degeneration it has been found that from 2 to 3 parts of water are used in order to get a glue sufficiently fluid for general application. If more water is added to make the glue more fluid, or it is rendered more fluid by other means, so that it might be commercially applied by hand brush or machine for joint work, then, when the glued surfaces are pressed together in the usual manner, it is found that so much of the glue is forced into the wood, due to its fluidity, that insufficient is left on the surface to make a desirable joint and, furthermore, the large amount of water so wets the wood that a much longer time is required for drying out, a disadvantage quite serious in most commercial practice. If such fluid vegetable glue be applied to wood veneers, and especially thin veneers, much the same difficulties are encountered, even if the glue be just as viscous as regular vegetable glue, but contains an excessive amount of water.

The object of my invention is to provide a process whereby these difficulties, attendant on the use of relatively fluid glues or glues containing a relatively large amount of water may be substantially overcome.

I find that when such dilute glues are applied and then promptly subjected to high pressure, as is done in commercial practice, the glue is forced deep into the pores of the wood, or much of it forced out side-

wise, or both, thereby preventing a desirable joint from being obtained. According to my invention, after the glue is applied, I allow it to stand without any pressure, or only slight pressure being applied for a time sufficient to permit a substantial amount of the water to dry out of the glue, before subjecting the glue of the joint to the relatively heavy pressure. By allowing the glue to stand before completing the pressure of the glue into the wood pores, the glue loses some of water to the wood or to the air, or both, and thickens somewhat, after which the relatively heavy pressure no longer causes excessive penetration or material squeezing out at the edges. I find that the water absorbed by the wood before the glue is pressed materially into the wood is more quickly dried out than is the water in the glue pressed into the wood. I find that the depth of penetration of the glue into the wood pores depends upon the fluidity of the minute portions of the glue which have already penetrated, and the pressure applied, and that the less the glue is forced into the wood, the quicker the wood will dry out, and that the less the glue is forced out sidewise, together with the less it is forced into the wood, the more glue is left between the wood surfaces to form the joint, although finally there must be sufficient penetration into the wood for the glue to take a firm hold thereon to form a secure joint. Thus during the first stage there is no material penetration of the glue into the wood and then when the relatively heavy pressure is applied the glue is only forced into the superficial pores of the wood sufficient to secure a good hold thereon, so that ample glue is left between the wood surfaces to form a strong joint.

The examples given below taken in connection with the accompanying sheet of drawings, will enable those skilled in the art to readily understand my invention and enable them to make use of the same.

In the drawings Figure 1 is an elevation of a press containing a stack of veneers with the glue applied thereto but without any substantial pressure being applied thereto. In the specific example illustrated they are merely subjected to the pressure of their own weight. The veneers are allowed to stand in this condition until a substantial part of the water has dried out of the glue

thereon. This illustrates the first step of the process. In Fig. 2 the second step is illustrated, in which the press is operated to apply pressure to further force the glue into the pores of the wood and the glue allowed to substantially dry out under pressure.

In the drawings core pieces are indicated at 1, 2, 3 and 4 with a layer of glue on each side thereof. Veneers 5 and 6 with a coating of glue applied thereto on the sides adjacent the core 1, are placed adjacent the core 1, as shown in Fig. 1. Veneers 7 and 8, 9 and 10, and 11 and 12 with similar glue coated surfaces are placed against the cores 2, 3 and 4 in the same manner, respectively, and the whole arranged to form a stack in the press, P.

After the necessary amount of water has dried out of the glue, pressure is applied to the stack as indicated in Fig. 2 and the glue forced into the superficial pores of the wood and further drying out is allowed while the layers are still under pressure.

Example 1: 100 pounds of corn starch are suspended in 343 to 368 pounds of water, and during constant agitation thereof 8 pounds of caustic soda dissolved in 32 pounds of water are slowly added, about 20 minutes being taken for the addition. The addition of the caustic soda causes the starch to be dissolved into a homogeneous colloidal glue. The stirring is preferably continued until the batch is used up, as standing tends to cause it to gelatinize. While this glue will flow readily through two inch pipes, the pipes should be cleaned of glue before being allowed to stand idle for any prolonged period, as for a day or more. The glue is preferably applied to both wood surfaces to be joined, but good results can be obtained by application to one surface only, and it gives better results if at least one of the wood members is greater than  $\frac{1}{2}$  inch in thickness. In order that the relatively large amount of water in the glue (3 $\frac{3}{4}$  to 4 parts by weight, per part of dry starch base) may not prove disadvantageous, the glued wood surfaces, after being placed in juxtaposition to one another, are allowed to stand for about  $\frac{1}{2}$  hour, with the pressure of their own weight merely, or without any substantial pressure being applied, so that a substantial part of the water will dry out of the glue before the glue is materially pressed into the wood, or before completing the pressure of the glue into the wood. Then a relatively heavy pressure, of 100 pounds per square inch may be applied to complete the pressure of the glue into the wood and the glue allowed to further dry out and set under such pressure.

In selecting the corn starch base, a starch having a viscosity of from 20 to 26 at 20 to 1 by Perkins viscosimeter, is preferred.

The Perkins viscosimeter may be constructed of brass tubing 1.295 inches outside diameter, 0.012 inch thick, and 3 inches long, and having a flat brass bottom 0.080 inch thick soldered into the end having a round center hole 0.070 inch in diameter, the total weight being 39.63 grams, and all edges being made smooth removing practically no weight, the hole being polished until the cup placed quickly at its floating level in water at 60° F. floats upright and fills up to the point of sudden sinking by top overflow in 16 seconds.

In making the viscosity test above described, about 350 grams of starch may be mixed with 20 times its weight of water and boiled for 10 minutes with dry live steam at 100 pounds pressure and tested for viscosity while at about 195° F. by placing the Perkins cup viscosimeter therein and measuring the number of seconds for it to sink by top overflow. When I speak of the viscosity being 20 to 26 at 20 to 1, I mean that it takes from 20 to 26 seconds for the cup viscosimeter to sink when the amount of water in the boil is 20 times the weight of the starch. When considerably more degenerated starches are tested, only 9 parts of water may be used, or 9 to 1.

In the example of glue above described, if slightly more water be used, as for instance, 4 $\frac{1}{4}$  parts instead of 3 $\frac{3}{4}$  parts, the glue will be rendered more fluid and more easily applied with a brush and used for joint work. In such case, however, it is desirable to allow a somewhat longer time for more water to dry out of the glue on the wood before applying the relatively heavy pressure to the glue joint.

Example 2: Good quality cassava starch is degenerated to a point such that it has a viscosity of about 40 at 9 to 1 when treated by the method above described. The degeneration may be accomplished in any suitable manner, as by the method described in U. S. Patent 1020656. 100 pounds of this degenerated starch is mixed with 700 pounds of water and 4 pounds of caustic soda added in a solution thereof containing 60 pounds of water. The caustic soda solution is added slowly while the temperature of the batch is raised to about 160° F. or somewhat less, and with continued agitation. When the batch has been transformed into glue and become clear, 25 pounds gum tragacanth, powdered to pass through a 60 mesh sieve, is added and stirred in while the temperature of the batch is maintained from 140° F. to 160° F. for 1 $\frac{1}{2}$  hours. This gives a relatively fluid glue, easily applied by a suitable brush, but owing apparently to the introduction of the gum tragacanth, the glue does not seem to penetrate the wood pores so readily as would be expected.

In applying this glue, and especially to

veneers, it is, however, preferable to allow the surfaces to be glued to remain in contact for about 3 hours without any substantial pressure being exerted on the joint, after which time a pressure of about 100 pounds per square inch or more may be applied until the glue is practically dry and set.

Example 3: 100 pounds of raw cassava starch having a viscosity of about 100 at 20 to 1, when tested as above described, is suspended in 368 pounds of water and 8 pounds of caustic soda, dissolved in 32 pounds of water, is gradually added with continued stirring, and the stirring preferably continued for about  $\frac{1}{2}$  hour after the caustic solution has all been added. The resulting glue is less viscous or more fluid than the glue produced when the degenerated starch base of Example 2 is dissolved in  $2\frac{1}{2}$  times its weight of water with the 8% of caustic soda. Also the glue is not particularly prone to gelatinize on standing if occasionally stirred, and after being applied to veneers, and the wood surfaces brought into juxtaposition, the veneers are preferably allowed to stand for about 20 minutes with less than 20 pounds per square inch pressure applied thereto, after which a pressure of 100 pounds per square inch or more may be applied.

30 The glue is more specially useful for heavy veneers and block work or core stock.

Example 4: 100 pounds of raw potato starch having a viscosity of 55 at 20 to 1 when tested by the method above described, are suspended in 280 pounds of water, and 4 pounds of caustic soda, dissolved in 20 pounds of water, are gradually added, with constant stirring, during a period of about 1 hour, during which time the temperature 40 of the batch is raised from 130° F. to a temperature from 150° F. to 160° F. The resulting glue is best applied warm and the pipes through which it is distributed kept heated to a little above 140° F. until 45 emptied. After the glue is applied to the wood, it should be allowed to stand 10 or 15 minutes without any substantial pressure being applied to the joint, after which the relatively heavy final pressure may be applied in the usual manner. However, if 50 the wood is hot, the time of standing should be increased to about  $\frac{1}{2}$  hour before the heavy pressure is applied.

Example 5: 100 pounds of raw cassava starch having a viscosity of about 80 at 20 to 1 when tested by the above described method, are mixed with 700 pounds of water, and 10 pounds of caustic soda, dissolved in 100 pounds of water, are slowly added with 60 constant stirring until the batch is transformed into a homogeneous solution, and then 30 pounds of gum tragacanth, powdered to pass through a 60 mesh to the inch sieve, are added and thoroughly stirred in 65 for about 2 hours. The resulting glue is

thin enough to be applied with a suitable brush, preferably a wire brush. After the glue is applied and the wood faces placed in juxtaposition to one another, the joints are allowed to stand for  $\frac{1}{2}$  hour under their own 70 weight, and then a pressure of 100 pounds per square inch is applied.

Example 6: The gum tragacanth may be introduced before the addition of the caustic, but the resulting glue in such case is 75 more fluid than if added afterward, other things being the same. For example, 100 pounds of the degenerated starch base of Example 2 and 25 pounds of gum tragacanth, powdered to 60 mesh, are suspended 80 in 350 pounds of water, and 4 pounds of caustic soda, dissolved in 30 pounds of water, are slowly added while the temperature of the batch is gradually raised to 150° F. to 160° F. with continual rapid agitation. The 85 rapid agitation is best continued until the glue is cold and the glue may be applied cold preferably to both faces to be joined. The glued surfaces should be allowed to stand for about 3 hours without material 90 pressure being applied to the joints, after which 100 pounds per square inch may be applied to the joints until the glue has practically set.

Instead of gum tragacanth, other highly 95 water absorbent material producing viscous solutions when mixed with water, may be used, as for instance viscose, or the xanthate of cellulose or xanthate of starch may be used.

Example 7: 100 pounds of cassava starch of good quality having a viscosity of about 90 at 20 to 1 when tested as above described, is suspended in 468 pounds of water and 8 pounds of caustic soda, dissolved in 32 pounds 105 of water, together with 10 pounds of carbon bisulfid, are slowly added during continued rapid agitation, until the batch comes across into a homogeneous glue solution. The stirring is preferably not unnecessarily prolonged thereafter. The starch is, I believe, put into the form of xanthate of starch. After the glue has been applied to the wood, it should be allowed to stand for about  $\frac{3}{4}$  hour without material pressure being applied to the joints, after which 100 pounds 115 per square inch pressure may be applied.

Example 8: A solution of sodium aluminate is first prepared by dissolving freshly precipitated aluminum hydroxid containing 120 about 15% actual  $\text{Al(OH)}_3$ , washed nearly free from salts, in the molecular quantity of caustic soda in solid form (about 96%  $\text{NaOH}$ ) to produce sodium aluminate. The solution should contain 22.3% of sodium 125 aluminate  $\text{Na}_3\text{AlO}_2$ . About 24.6 pounds of this solution containing about 5.5 pounds of  $\text{Na}_3\text{AlO}_2$  are added to 375 pounds of water and 100 pounds of the degenerated cassava starch base of Example 2 are then stirred in 130

and the temperature raised to about 160° F. until the suspended starch and water are transformed into a homogeneous adhesive solution. The stirring is then continued 5 until the batch is cold. If desired, the aluminum hydroxid may be added after the starch has been suspended in cold water containing the 3.5% of caustic soda and then the temperature raised to bring about solution, the liquid, upon the raising of the temperature, containing actually, or in effect, 10  $\text{Na}_3\text{AlO}_3$ . Sometimes it is desirable to add about 10% more of the  $\text{Na}_3\text{AlO}_3$  than above indicated. After the glue is applied to the 15 wood, it should be allowed to stand for a substantial period without materially pressing the glue into the wood to allow a substantial part of the water to dry out of the glue after which the final pressure may be 20 applied to the joint to complete the pressure of the glue into the wood.

Example 9: Good quality cassava starch is degenerated to a point where its viscosity is about 60 at 9 to 1, when tested by the 25 method above described. The degeneration may be carried out by any suitable method, such as by the degenerating agents specified in U. S. Patent 1020656. 100 pounds of this degenerated starch base are mixed with 368 30 pounds of water and 3 pounds of caustic soda, dissolved in 32 pounds of water, gradually added during twenty minutes, with continual agitation, and while the batch is kept at about 145° F. The resulting glue 35 may be used hot or cold, but after application to the wood, the surfaces to be glued are placed adjacent one another and slight pressure applied, but insufficient to cause the glue to be materially pressed into the wood pores. After about  $\frac{1}{2}$  hour, the pressure is 40 increased to complete the pressure of the glue into the wood pores and the glue is permitted to further dry out and set under this increased pressure.

Example 10: Good quality raw cassava starch having a viscosity of 90 to 100 at 20 to 1 when tested as above described, is mixed with twice its weight of water, and while being agitated  $\frac{1}{2}\%$  (based on dry weight of 50 the starch) of caustic potash in 10% solution in water is added. There is also added about the same time, from  $\frac{1}{4}\%$  to 1% of sodium peroxid in 5% solution in water. The mixture is agitated for about 12 hours 55 or more, until the starch has been degenerated to a point where its viscosity is from 24 to 26 at 9 to 1 when tested as above described. The percentages of reagents added may be varied somewhat to bring about the 60 desired amount of degeneration. The starch glue base is then further treated with  $\frac{1}{4}\%$  sodium peroxid and  $\frac{1}{4}$  to  $\frac{1}{2}\%$  caustic potash, in solution as before, the addition being made slowly and with continual stirring to 65 prevent the local bursting of the suspended

starch particles, and the stirring continued for several hours until the viscosity of the starch is about —26— at 9 to 1 when tested as above described. Or the starch may be removed from the alkaline liquor and again 70 suspended in 2 parts of water and  $\frac{1}{4}\%$  of sodium peroxid and  $\frac{1}{4}\%$  of caustic potash and the starch given a second treatment substantially like the first. In either case, the final viscosity of the starch is reduced to 75 about —17— at 9 to 1.

The starch is finally removed from the alkaline liquor and dried and 100 pounds thereof suspended in 150 pounds of water and 16 pounds of caustic potash, dissolved 80 in 48 pounds of water, added slowly with constant stirring, until the mixture is dissolved into glue.

Instead of degenerating the starch as above described, it may be degenerated by 85 any other reagents or method or a starch of the proper viscosity selected, and then dissolved with the caustic potash as above described. If heat up to 150° F. is used in the dissolving step, the percentage of caustic 90 potash used may be considerably reduced.

The resulting glue is very permanent, and in spite of the small quantity of water therein, is also very fluid and capable of ready application by a suitable brush for joint work. 95 However, after being applied to the wood, it should be allowed to stand 15 or 20 minutes before very high pressure is applied.

From the above, it will be seen that by my invention, especially in its broader aspects, 100 many glues containing a relatively large amount of water, or being very fluid, or both, are made commercially applicable and the disadvantages hereinbefore mentioned are substantially overcome. I have found 105 that a gradual and at first low increase of pressure is in all cases equally good, if properly regulated, as will be apparent from the above examples, to anyone skilled in the art, after a few trials, and, in some cases, this 110 method has the advantage of bringing all parts of the glued surfaces earlier into contact without exerting excessive pressure upon the mass of the glue. Hence, I desire to cover all modifications and forms coming 115 within the language of the appended claims.

What I claim as new and desire to secure by Letters Patent, is:

1. In the improved process of gluing wood, the steps which consist in applying 120 to wood a water containing glue made from a starchy carbohydrate base and allowing the glue to remain on the wood for a substantial time without material penetration of the glue into the wood and before completing the pressure of the glue into the superficial wood pores to permit 125 a substantial part of the water in the glue on the wood to dry out of the glue before completing the pressure of the glue into 130

the superficial pores of the wood and then pressing the glue farther into the pores of the wood.

2. In the improved process of gluing wood, the steps which consist in applying to the wood a glue containing a starchy carbohydrate base and about four parts or more by weight of water and allowing a substantial part of the water in the glue 10 on the wood to dry out without material penetration of the glue into the wood and before pressing the glue materially into the superficial pores of the wood, and then applying pressure to the glue joint to force 15 the glue farther into the superficial pores of the wood and allowing the glue to further dry out under pressure.

3. In the improved process of gluing wood, the steps which consist in applying 20 to the wood a glue containing a starchy carbohydrate base and water and allowing a substantial part of the water in the glue on the wood to dry out without material penetration of the glue into the wood and 25 before pressing the glue materially into the pores of the wood and then applying pressure to the glue joint to force the glue farther into the pores of the wood and allowing the glue to further dry out under pressure.

4. In the improved process of gluing together layers of wood, the steps which consist in applying to one or both wood surfaces to be joined a glue containing a 30 starchy carbohydrate base and water, then placing the wood surfaces to be joined in juxtaposition to one another and under a pressure of about 10 pounds per square inch or less for a period sufficient to permit

a substantial part of the water to dry out 40 of the glue and without material penetration of the glue into the wood and then increasing the pressure to about 100 pounds per square inch or more and allowing the glue to further dry out under such increased pressure.

5. In the improved process of gluing together layers of wood, the steps which consist in applying to one or both wood surfaces to be joined a glue containing a 50 starchy carbohydrate base and water, then placing the wood surfaces to be joined in juxtaposition to one another and allowing a substantial part of the water in the glue on the wood to dry out of the glue without 55 material penetration of the glue into the wood and before completing the pressure of the glue into the wood pores and then applying pressure to the glue joint to force the glue farther into the pores of the wood 60 and allowing the glue to further dry out under pressure.

6. In the improved process of gluing wood, the steps which consist in applying to the wood a water containing glue and 65 allowing a substantial part of the water in the glue on the wood to dry out of the glue without material penetration of the glue into the wood and before completing the pressure of the glue into the wood pores 70 and then applying pressure to the glue joint to force the glue farther into the pores of the wood and allowing the glue to further dry out under pressure.

Signed at New York city, in the county 75 of New York and State of New York this 15th day of January A. D. 1918.

WILLIAM M. GROSVENOR.